

## [54] PRESSURE FIXING OF TONERS

[75] Inventors: **Richard S. Brenneman**, Natick; **David W. Lovering**, Needham, both of Mass.; **Frederick E. Barr**, Vermillion, Ohio

[73] Assignee: **Addressograph-Multigraph Corporation**, Cleveland, Ohio

[22] Filed: Mar. 12, 1973

[21] Appl. No.: 340,600

## Related U.S. Application Data

[63] Continuation-in-part of Ser. No. 51,089, June 30, 1971, abandoned, which is a continuation of Ser. No. 694,515, Dec. 29, 1967, abandoned.

[52] U.S. Cl. 117/21, 29/132, 117/17.5, 118/637, 118/114

[51] Int. Cl. G03g 13/20, G03g 15/20

[58] Field of Search 117/9, 16, 17.5, 21, 118/114, 116, 117, 637; 219/216, 388, 469, 470; 226/177, 181; 29/132

## [56] References Cited

## UNITED STATES PATENTS

|           |         |                  |          |
|-----------|---------|------------------|----------|
| 3,501,823 | 3/1970  | Gregersen et al. | 29/132   |
| 3,617,445 | 11/1971 | Brafford         | 162/358  |
| 3,269,626 | 8/1966  | Albrecht         | 226/177  |
| 3,307,993 | 3/1967  | Gottwald et al.  | 117/65.2 |
| 3,331,592 | 7/1967  | Cassano et al.   | 219/388  |

|           |         |                 |          |
|-----------|---------|-----------------|----------|
| 3,338,735 | 8/1967  | Hain            | 117/65.2 |
| 3,398,011 | 8/1968  | Neirotti et al. | 118/114  |
| 3,449,548 | 6/1969  | Adamek et al.   | 219/388  |
| 3,345,937 | 10/1967 | Kusters et al.  | 29/132   |
| 3,511,729 | 5/1970  | Williams        | 29/132   |
| 3,637,416 | 1/1972  | Misch et al.    | 29/132   |
| 3,753,276 | 8/1973  | Reisch          | 29/132   |
| 1,055,404 | 3/1913  | Kremmer         | 118/117  |
| 2,711,985 | 6/1955  | Olson           | 117/21   |
| 2,852,412 | 9/1958  | Hassel          | 118/114  |
| 2,859,673 | 11/1958 | Hix et al.      | 117/17.5 |
| 2,955,052 | 10/1960 | Carlson et al.  | 117/21   |
| 3,013,526 | 12/1961 | Crumrine et al. | 117/17.5 |
| 3,063,859 | 11/1962 | Heckscher       | 117/17.5 |
| 3,071,070 | 11/1963 | Matthews et al. | 117/17.5 |
| 3,093,068 | 6/1963  | Gundlach et al. | 117/17.5 |
| 3,094,429 | 6/1963  | Howell          | 117/17.5 |
| 3,268,351 | 8/1966  | Van Dorn        | 117/21   |

Primary Examiner—Michael Sofocleous

[57]

## ABSTRACT

A method of fixing toners to a surface without the use of heat employs pressure which is applied by two somewhat compliant rolls, or one somewhat compliant roll and one relatively rigid roll. The use of such an arrangement makes it possible to apply a substantially uniform pressure to the toned areas to secure a uniform fixing action throughout.

21 Claims, 3 Drawing Figures



PATENTED DEC 17 1974

3,854,975

SHEET 1 OF 2



Fig. 1



Fig. 2

INVENTORS.

RICHARD S. BRENNEMAN

DAVID W. LOVERING

FREDERICK E. BARR

BY *Russell L. Root*  
ATTORNEY

PATENTED DEC 17 1974

3,854,975

SHEET 2 OF 2



Fig. 3

INVENTORS.  
RICHARD S. BRENNEMAN  
DAVID W. LOVERING  
FREDERICK E. BARR

BY *Russell L. Post*  
ATTORNEY

**PRESSURE FIXING OF TONERS**

This application is a continuation in part of application Ser. No. 51,089 filed June 30, 1970, now abandoned which in turn is a continuation of application, Ser. No. 694,515, filed Dec. 29, 1967 now abandoned.

**STATEMENT OF BACKGROUND AND OBJECTS**

The process of copying indicia by the technique of forming an electroscopic powder on a surface of a substrate material is well developed. Typically, this is accomplished in either of two ways. In either of these methods, a photoconductive surface is electrically charged and then exposed to a light and shadow pattern of the image. The electrostatic charge which was deposited upon the photoconductive surface is removed from those places exposed to light, leaving a latent electrostatic image which can be developed. Development is accomplished by exposing the electrostatic image to a colored powder, usually referred to as a "toner" in this context, having the property of being attracted to the electrostatic image areas. According to the first method, the toner is then fixed (permanently adhered) to the photoconductive surface. According to the other method the toner image formed on the photoconductive layer is first transferred to another substrate, e.g., a sheet of ordinary paper, and is then fixed on that other substrate.

In addition to the typical processes above described, it will be readily appreciated that other techniques for depositing toner particles on a substrate under the control of an electrostatic image pattern have been developed, and any of these are usable in conjunction with the fixing technique described in detail hereinafter.

The toner is normally a blend of thermoplastic resin, carbon black or other pigment, and a small amount of dye. The exact composition depends upon the specific purpose for which it is to be used.

The fixing or adhering of the toner is normally accomplished by heat fusing the thermoplastic resin component thereof. This is usually performed by exposing the image to heat for a time sufficient to melt somewhat the toner particles so that they adhere, one to the other, and to the paper or substrate. Some fixing techniques have also employed the pressure developed by two hard surfaced rolls to fix the particles. Another proposed process passes the substrate between hard surfaced rolls in combination with the application of heat.

Heat fusing, while producing effective results in many cases, is undesirable in that it requires that a supply of heat be available, usually entailing a supply of electric power in large quantities, and presents the possibility of overheating the substrate as well as the toner, with some danger of fire as a result. Pressure fixing as applied in the prior art has consisted of passing the toned substrate between two hard surfaced rolls, formed of metal, one roll being movable and connected with springs to provide a controlled pressure. (See for example U.S. Pat. No. 3,269,626). Experience has shown that this type of pressure fixing proves very unreliable, possibly due to poor contact because of non-uniformity of the substrate thickness, variation in the toner deposit, or the like, even though use is made of extremely high loadings in an effort to obtain an image adequately adhered in all of its portions. This is particularly true if wider sheets are used rather than tapes. Under high loadings the character of the paper substrate itself may be materially altered, for to apply enough pressure to the low points or areas in the paper

to properly fix the toner, it is necessary to apply excessive pressures to the high points. This, in turn, can materially alter the substrate and bring about unwanted surface characteristics in the unprinted areas, i.e., make certain areas shiny or glossy rather than permitting them to remain dull, and in any event almost certainly fails to provide degrees of fixing in various portions of the sheet which are sufficiently uniform to be practical in most applications.

It is perhaps theoretically possible, if the destructive effect upon the sheet could be neglected, to urge the rollers together with sufficient force to provide general and fairly uniform fixing of the toner on a sheet of ordinary size, for example 8½ inches by 11 inches. The difficulty, however, is, that the loading required in such a situation may well transcend the normal range by such a large amount that the mechanical elements of the system (such as the rollers themselves and their load-applying bearings) would either fail directly under the applied load, or would deteriorate so rapidly due to fatigue that no practical device could be constructed to accomplish this end within the framework of normal economic realities.

It is therefore a primary object of this invention to provide an improved method for pressure fixing toners to a substrate without the use of heat. It is another object to provide a method which supplies a substantially uniform pressure to the toned areas without adversely affecting portions of the substrate. It is another object of the invention to provide an arrangement or narrow band, progressive contact, pressure members for pressure fixing a toner to a substrate, which pressure members have properties such that they can produce an effective uniform fixing action on a substrate sheet of normal size under reasonable loading forces, thus permitting the design of a practical machine without introducing undue design difficulties. Other objects of the invention will in part be obvious and will in part be apparent hereinafter as the description proceeds.

For a fuller understanding of the nature and objects of the invention, reference should be had to the following detailed description taken in connection with the accompanying drawings in which:

FIG. 1 is a perspective representation of the apparatus for carrying out the pressure fixing method of this invention including, in combination, in block diagram form, the apparatus for accomplishing the customary precedent steps of charging, exposing, developing, and in some cases transferring;

FIG. 2 is an enlarged side elevation of the pressure fixing portion of the apparatus shown in FIG. 1 with the loading and driving means omitted; and

FIG. 3 is a diagrammatic side elevation to a larger scale showing cylinders in relaxed engagement and in pressure engagement, and illustrating the meaning of certain symbols used in the description.

**DESCRIPTION OF THE PREFERRED EMBODIMENT**

Referring to FIG. 1, the process of forming the powder image is carried out in the usual manner wherein a member or sheet carrying a photoconductive layer is automatically fed past a charger 3 to receive a uniform static charge on its surface, is then automatically fed to an exposure station 4 where it is exposed to a light and shadow pattern corresponding to the desired image, then is automatically fed to developer equipment 5 where the latent image is developed with a toner powder according to known procedures and finally fed directly (as by path 6) to a fixing station 10. In the alternative, a latent electrostatic image similarly formed on

the photoconductive layer of a member or sheet may be developed with toner, and the toner image thus formed transferred therefrom to another sheet or substrate as both are fed automatically (as by alternate path 7) through a transfer station 8. In any event, the resulting product is a flexible sheet or substrate 11 with a loosely held image 13 defined by toner powder on its surface, being automatically fed to a fixing station 10.

In accordance with the invention herein the substrate carrying the toner image is then passed through the said fixing station 10 which comprises pressure members which progressively contact each other along a line of narrow band area, and emerges with the image consolidated and firmly adhered to the substrate as at 13'. Normally, these pressure members consist of a roll and an opposing member in rolling pressure contact therewith. In the most convenient arrangement, this opposing member is also a roll.

In the preferred form illustrated in the drawing there are two rolls 15 and 17 forming a nip into which the toner bearing sheet 11 is passed. In accordance with prior practice these rolls would be hard metal rolls, but in accordance with the present invention it has been discovered that at least one of these rolls or members should be of softer, more compliant material. From a basic fixing standpoint, both members or rolls could be equally compliant or deformable. However, from the standpoint of effective practical operation, it is found that it is usually easier to provide a toner rejecting surface on a hard, relatively rigid, member. Accordingly, the upper roll 15 in contact with the toner image is preferably a hard surfaced metal roll, and the lower roll 17 is of a softer and more compliant material.

The more compliant roll may be of any material which has a certain amount of resiliency associated with its surface. Thus, for example, it may be formed of a hard rubber, it may be a cloth filled or a paper filled roll, it may be formed of such materials as corn cobs or asbestos, or may be of any of various resilient synthetic resinous materials of appropriate hardness and deformability, nylon and acetal resin (sold under the trademark DELRIN) being examples. A number of types of such resilient rolls are known in the papermaking art for various purposes unrelated to the instant problem. The form of compliant roll presently preferred is one which is made up of stacked sheets of textile embodying cotton fibers and wool fibers in approximately equal amounts. The more compliant roll must generally have a central metal shaft (e.g., steel) covered with a layer of the more compliant material, which layer is usually effective for the purposes of the invention when the thickness of the layer is one-fourth or more. Accordingly when the description speaks about rolls of compliant material, such composite rolls are understood to be included.

As the toned substrate 11, 13 passes between the rolls 15 and 17, the surface of the compliant roll 17 apparently becomes slightly distorted, as seen in exaggerated representation at 19 in FIG. 2, so that pressure is distributed over a wider part of the substrate. Moreover, the more compliant characteristic of the roll 17 makes it possible for the roll to adjust to variations in the thickness of the paper substrate or the toner deposit, and thereby distribute the pressure more evenly, making it possible to effect application of a substantially uniform pressure to areas containing the toner image which is to be fixed. It is possible that in passing

between the rolls, some shear is developed which contributes to the fusing of the toner to the paper. However, it is believed that the application of a uniform pressure to the toner is probably the primary factor in the achievement of good toner fixing.

In passing the toner bearing substrate into the nip of rolls 15 and 17, it is desirable that the toned side be brought into contact with the relatively rigid roll 15. This results in better pressure fixing to the substrate surface and in the prevention of toner build-up on the more compliant roll surface. This latter factor is particularly important where the surface of the more compliant roll possesses any degree of porosity, for the finely divided toner could gradually build up in the surface pores. The relatively rigid roll is preferably of a material whose surface is smooth and non-porous, and which has the property of resisting adhesive attachment for the resins employed in the toner particles. Chrome plated steel is generally quite effective for this purpose.

When the toned surface is faced towards the relatively rigid roll as described above, the substrate must, of course, be of a rather flexible nature to permit the action of the more compliant roll to have its desired effect.

In the drawing, the compliant roll 17 is shown as having a larger diameter than the relatively rigid roll. This is normally desirable but not necessary. Whether the two rolls are of the same or different size, they are rotated so as to have essentially the same surface speed. This means that the shear developed, if any, will be due almost solely to the surface characteristics of the more compliant roll.

The loading to be applied to the rolls or pressure members 15 and 17 may be effected by joint loading and driving means of conventional character indicated diagrammatically at 21 in FIG. 1, and varies with a number of factors such as the resilience of the members and the pressure response level of the toner. The initial tests conducted in connection with this discovery were performed using a cotton filled roller of a hardness on the Shore-D scale of about 80 and having a calculated modulus of elasticity in compression of about 200,000 p.s.i. operating against a steel-roller. It was found that many conventional toners were effectively fixed to the substrate when the loading was in the range of about 200 pounds to 400 pounds per lineal inch. The toners used in these tests were conventional dry toners embodying as the binding agent the resins customarily used heretofore for this purpose. A calculation of the peak pressure which the rollers could be said to apply, on an average, at the incremental area of their contact gives about 5,000 to 10,000 p.s.i.

These figures represent a particular example of a rather usual situation in which the invention can be applied, but it will be understood that the loading of the pressure members can be adjusted to give the desired pressure, depending upon the rigidity of the roll material used, and that the pressure may be varied substantially to meet the fixing requirements of the particular toner.

Other tests were conducted using a nylon roller in place of the cotton filled roller, and then using a second nylon roller in place of the steel roller, to provide two relatively compliant rollers operating against each other. For purposes of calculations, the modulus of elasticity in compression for the nylon rollers were deemed to be 400,000 p.s.i. based on the manufac-

er's information that the modulus was in the range of about 350,000 p.s.i. to about 450,000 p.s.i.

Some of the toners used in these additional tests were extremely soft, being fixable at cylinder loadings at as low as 50 p.l.i. in a nylon-steel roller system. Other toners used were moderately soft, being fixable at cylinder loadings of about 150 p.l.i. in a nylon-steel roller system.

Calculated peak nip pressures ranged from about 2,000 p.s.i. for very soft toners fixed between two nylon rollers to about 3,000 p.s.i. for the same toners fixed between one steel and one nylon roller; and from about 3,800 p.s.i. for moderately soft toners fixed between two nylon rollers to about 5,300 p.s.i. for the same toners fixed between one steel and one nylon roller.

Absolute peak nip pressure values it should be noted are not delimitative of the scope of the invention. However, it may be helpful to point out for the purpose of general understanding of the background of the invention that values within the range of about 2,000 p.s.i. to 10,000 p.s.i. are the ones which would be more frequently encountered in the practice of the invention. Based on the complete discussion presented herein, it will be apparent to those acquainted with the art that the inventive concept involves the use of one or more compliant rollers to apply the requisite fixing pressure as opposed to mating hard-surfaced rollers as was heretofore thought to be essential. Specifically, even if an effective toner having a threshold pressure equivalent to 1,000 p.s.i. peak at the roller nip, or less, was available, the novel concept of using at least one compliant roller to provide heatless fixing would still provide the key to success if the system exhibits the appropriate deflection at the pressures used and discussed in detail hereinafter.

While the particular resilient rollers described above had calculated moduli of elasticity within the range of about 200,000-450,000 p.s.i., it will be understood that other resilient materials can be used in applying the invention and having a modulus much higher than 450,000 p.s.i. based on principles to be explained hereinafter. As to the minimum modulus, it should be such that the material does not deform excessively. Usually a calculated modulus of at least 100,000 p.s.i. is considered preferable in the best interests of over-all efficiency. With the usual conditions, and working against a steel roll, the maximum effective value for the modulus of the more compliant roll will usually be found to be about 2,000,000 p.s.i.

As a basis for comparison it may be noted that the modulus of elasticity for steels is close to 30,000,000 p.s.i.

The immediately foregoing statements will perhaps be more readily understood in the light of the following comments.

The mechanical interaction of two parallel cylinders urged against one another has been extensively investigated and mathematical relationships developed which will permit the calculation of quantities such as (a) an apparent calculated value for the modulus of elasticity for the cylinder material (where, for example, the material is of a type not having a commonly recognized or recorded modulus value), and (b) the maximum compressive stress or peak effective pressure in p.s.i. exerted by the cylinders at the nip. An example of these relationships can be found in Formulas for Stress and

Strain (Fourth Edition) by Raymond J. Roark, published by McGraw-Hill Book Company.

On page 320 of the Roark text, table XIV, Section 5, is found the expression:  $b = 1.6 \sqrt{D_1 D_2 / (D_1 + D_2)}$  [1 -  $V_1^2 / E_1 + 1 - V_2^2 / E_2$ ]

where:

$b$  represents the transaxial width in inches of the contact area under load (See FIG. 3);

$p$  represents the cylinder loading in pounds per lineal inch;

$D_1$  and  $D_2$  represent the diameters of the cylinders in inches;

$V_1$  and  $V_2$  represent Poisson's ratio in compression for the materials of the cylinders; and

$E_1$  and  $E_2$  represent the modulus of elasticity in compression for the materials of the cylinders, stated in pounds per square inch.

From this it will be seen that when a measurement is taken of the quantity  $B$  (as by loading the rolls with a pressure transfer material and a copy sheet therebetween and measuring the breadth of the print) and if one of the rolls has an  $E$  of known value (such as steel), the  $E$  (calculated modulus of elasticity) for the other roll can be readily obtained. (The effective value of Poisson's ratio for materials in the usable range may be assumed to be closely in the neighborhood of 0.3 in case there is no value reported in the literature, especially since this quantity has little effect on the calculated result).

At the same point in the text identified above, there is also found the expression:

$$\text{Max. } s_c = 0.798 \sqrt{p [(D_1 + D_2) / D_1 D_2]} / (1 - V_1^2 / E_1 + 1 - V_2^2 / E_2)$$

Where Max.  $s_c$  represents the maximum compressive stress or peak unit pressure effect at the nip, expressed in p.s.i., and the other symbols have the same significance as above. As will be readily seen, this formula gives the calculated peak nip pressure directly by merely substituting the appropriate values for  $p$ ,  $D_1$ ,  $D_2$ ,  $E_1$ ,  $E_2$  and the reported or assumed values for Poisson's ratio.

The significance of certain of the foregoing symbols will perhaps be more clearly understood by reference to FIG. 3 which shows two cylinders which may be considered as corresponding to rolls 15 and 17 of FIGS. 1 and 2. In the full line position the cylinders are unloaded, and the axis of cylinder 15 is at A. In the dotted line position the cylinders are under an applied load  $p$  which causes the axes to move closer together as represented by the shift of the axis of 15 to B. The distance AB or  $y$  can be measured and is referred to as the deformation. The loaded cylinders demonstrate a narrow band of contact under load having a width  $b$  which can be measured as heretofore described. Similar calculations can be made if either member becomes a plane by letting the value for the diameter of that member approach infinity in the above expressions, in which case  $D_1 D_2 / D_1 + D_2$  approaches D.

The tests conducted in connection with this invention have indicated that a certain calculated peak pressure at the nip is needed to secure proper fixing of a given toner, and that this is related primarily to the character of the toner material. As previously stated, for conventional toners currently in use, i.e., those requiring a cylinder loading of about 200 to about 400 pounds per linear inch, a calculated peak pressure of at least 5,000

p.s.i. is needed to secure fixing while for very soft toners, peak nip pressures as low as about 2,000 p.s.i. surface. The fixing here contemplated involves essentially altering the state of the toner resin sufficiently to make it flow and adhere to itself and to the substrate. This is, presumptively, primarily due to a pressure-induced temperature rise with the toner material although mechanical action may play a minor role in the fixing action also. Toners requiring a lesser pressure have been developed and may be used in the practice of the present invention. Examples of soft toners, fixable with only nominal pressure are disclosed in Canadian Pat. No. 874,011 issued July 6, 1971 to the assignee of the present application. It is also conceivable that in compounding toners to secure other beneficial properties, the pressure threshold might have to be increased. In any event, there will be a readily determinable minimum effective value of pressure for the particular toner under consideration, and that value will be referred to hereinafter as the threshold pressure for the toner.

Testing with exemplary moderately soft and conventional toners produced the following results:

| Ingredient                                    | Example I | Wt. % |
|-----------------------------------------------|-----------|-------|
| Hexanamide                                    | 46        |       |
| Hydroxylated fatty acid                       | 10        |       |
| Paraffin wax                                  | 30        |       |
| Nubian resin black                            | 12        |       |
| Carbon black pigment<br>(Neo-spectra-Mark II) | 2         |       |

The above toner composition was prepared in accordance with procedure described in the aforesaid Canadian Pat. No. 874,811 and deposited in a predetermined pattern on a lithographic master. The toned master was then passed between a steel and a nylon roller set at a cylinder loading of 50 p.l.i. Using the formula described above, a peak nip pressure was calculated to be 3,067.8 p.s.i. The level of fixing, as evaluated by measuring the optical density of toner transferred from the master to a cloth square utilizing a Crockmeter CM-5 instrument (Atlas Electric Devices, Chicago, Illinois) was deemed to be very good.

| Ingredient                                                                                                            | Example II | Wt. % |
|-----------------------------------------------------------------------------------------------------------------------|------------|-------|
| Sodium Stearate                                                                                                       | 50         |       |
| Acrawax C                                                                                                             | 20         |       |
| A synthetic wax — octadecanamide<br>(mp 140-143°C) manufactured by<br>Glycol Products Company, Brooklyn,<br>New York. |            |       |
| Tetradecanoic Acid                                                                                                    | 20         |       |
| Nubian Resin black                                                                                                    | 10         |       |

The foregoing composition was processed as in Example I and the resulting toner deposited on a lithographic master, also as described in Example I. The level of fixing at a cylinder loading of 50 p.l.i. was deemed to be good.

### EXAMPLE III

The procedure of Example I was repeated with the following composition except that the cylinder loading was set at 150 p.l.i.:

| Ingredient           | Wt. % |
|----------------------|-------|
| Acrawax C            | 90    |
| Nubian Resin black   | 5     |
| Carbon black pigment | 5     |

Using the formula described above, a peak nip pressure was calculated to be 5313.6 p.s.i.

10 The level of fixing achieved was deemed to be excellent.

15 The procedure of Example III was repeated using the following composition:

| Ingredient                                    | Wt. % |
|-----------------------------------------------|-------|
| Acrawax C                                     | 24    |
| Carnauba Wax                                  | 20    |
| 9-octadecanamide                              | 41    |
| Nubian Resin black                            | 10    |
| Carbon black pigment<br>(Neo-spectra-Mark II) | 5     |

25 Again, the level of fixing attained was deemed to be excellent.

| Ingredient                                                              | Example V | Wt. % |
|-------------------------------------------------------------------------|-----------|-------|
| Sucrose benzoate                                                        | 55.6      |       |
| RX 281 (Monsanto)<br>(Maleic anhydride-styrene<br>copolymer-half ester) | 11.1      |       |
| Elvaz 210 (DuPont)<br>(Ethylene-vinyl<br>acetate copolymer)             | 3.3       |       |
| AC 680 (Allied Chemical)<br>(Polyethylene)                              | 8.9       |       |
| Polywax 2000 (Bareco Chem.)                                             | 13.3      |       |
| Irgacet black RL<br>(Ciba-Geigy)                                        | 5.6       |       |
| Mogul L (Cabot Corp.)                                                   | 2.2       |       |

30 A toner having the above composition was deposited on Hammermill Xerocopy 10300-2 paper in accordance with predetermined pattern.

35 The toned sheet was then passed through a pressure fixing unit consisting of two nylon rollers operating against each other at a cylinder loading of 363 p.l.i. A peak nip pressure was calculated at 5,885 p.s.i. The level of fixing was deemed to be very good.

40 The parameters involved in securing adequate uniform fixing appear, from the tests so far conducted, to be substantially as described hereinafter.

45 The materials for the purpose members or rolls are (or where, as in the preferred example, one roll has significantly more "give" or compliance than the other, the material for the compliant member or roll is) selected to have values (or a value) of the modulus of elasticity such that, when a loading  $p$  is applied which generates a calculated peak nip pressure (Max.  $s_c$ ) equal to or slightly greater than the threshold pressure for the toner under consideration, there is generated a measured deformation ( $y$ ) which is still within the elastic limit for the material and whose value is a substantial multiple of the average variation in the workpiece properties. By this variation is meant variation in anything which offers resistance to squeezing, such as

50

55

60

65

thickness or density. For practical purposes, a standardized pressure is usually applied in taking such thickness measurements, so that the overall effect may normally be regarded as a thickness variation even though a density or compressibility factor may contribute somewhat thereto. Ordinary paper sheets, to take a convenient example, exhibit variations on the order of 0.0004 inches between the maximum and minimum thickness readings. While the thickness of the toner deposit can, under some circumstances, contribute to this variation and then might need to be taken into account, for most current toner materials and their usual depositing characteristics, be neglected in computing the thickness variation. It is contemplated, however, that situations involving very uniform substrates and toners exhibiting variations in particle size would respond equally to the methods and apparatus proposed herein, so that when a workpiece thickness variation is referred to hereinafter, this form will be understood as included as well as formed of workpiece variation arising primarily from substrate nonuniformity.

For purposes of convenience, variations of this sort which appear as a result of thickness measurement tests may be referred to as "thickness variations."

The term "substantial multiple," used in the immediately foregoing paragraph, means at least several times, and in practical effect, it has been found that, when the calculated peak pressure at the nip is at or slightly above the threshold pressure of the toner, a multiplier of about five, as a minimum, should be applied to the average variation to determine the appropriate deformation in order to secure reasonably uniform fixing on the surface of the substrate. A more generally preferred value would be a multiplier of 10.

This multiplier does not have a firmly fixed value or range, however, but probably depends to some extent on the amount by which the calculated peak nip pressure used is permitted to exceed that required for the toner in question.

Thus, for a toner whose threshold pressure is 5,000 p.s.i., and having in mind an ordinary paper sheet with an average thickness variation of about 0.0004 inches, the material of the roll 17 would be so selected as to its modulus of elasticity (E) that, when loaded to a value  $p$  which will give the calculated peak nip pressure of 5,000 p.s.i. required, or a little more, the measured deformation  $y$  should be at least  $5 \times 0.0004$  or 0.002 inches. As pointed out above, this might prove somewhat marginal, and the E would preferably be so selected that a deformation  $y$  of about  $10 \times 0.0004$  or 0.004 inches can be achieved to insure absolute fixing uniformity. However, if we should use a loading  $p$  which would produce a calculated peak nip pressure rather greater than is needed for the toner in question, say 15,000 to 20,000 p.s.i., and if this could be used without damaging the substrate, then it is expected that the deformation generating multiple applied to the average variation could be permitted to have a lesser value, perhaps in the range of 3 to 4 as a minimum.

From the foregoing discussion it will be apparent that having the threshold pressure of the toner in mind, and the average variation in workpiece properties (represented as a thickness variation) it is possible to determine readily whether any particular solid material of a coherent elastic nature will have the properties needed to form an effective pressure fixing member. For convenience it may be stated that the pressure members or

rolls will be of a material having a modulus of elasticity in compression such that, when subjected to a loading which develops a calculated peak nip pressure of at least the threshold pressure of the toner in question, they will exhibit a deformation which is a substantial multiple of the workpiece thickness variation.

It will be understood that, while the two roll form has been shown and described, either pressure member may be formed as a platen with the other having a roll or segment configuration and being in rolling pressure contact therewith.

Most of the powdered toners now commonly known and used may be used in forming copies by the process of this invention. However, since the method of this invention achieves uniform toner adherence to the substrate surface by application of pressure alone, it presents an opportunity to use other finely divided powders for toners which are not necessarily the same as those usable in heat fusing. Thus, a greater flexibility in toner choice and final copy characteristics is available.

The method of pressure fixing of this invention makes it possible to work with wider substrate sheets than is possible with the use of two hard surface rolls. Past experience in using two hard surface rolls has indicated that problems of achieving satisfactory characteristics in the untoned surface areas are materially increased as the width of the substrate is increased. This intensification of the fixing problem with increase in width is not experienced when fixing is effected in accordance with the procedure set out in the foregoing description.

It will thus be seen that the objects set forth above, among those made apparent from the preceding description, are efficiently attained and since certain changes may be made in carrying out the above method, without departing from the scope of the invention, it is intended that all matter contained in the above description shall be interpreted as illustrative and not in a limiting sense.

While preferred embodiments of the invention have been described and illustrated, it is to be understood that these are capable of variation and modification. Accordingly, the aim in the appended claims is to cover all such variations and modifications as may fall within the true spirit of the invention.

What is claimed is:

1. The method of providing a permanent image on a substrate of substantial width, wherein the image is a fixed powder image of electroscopic toner powder having a predetermined threshold pressure, comprising the steps of creating an electrostatic charge pattern in image configuration; depositing electroscopic toner powder upon said substrate to form an image pattern configuration under the electrical control of said charge pattern to create a workpiece having thickness variations; and fixing the toner powder image to said substrate, wherein the last mentioned step includes providing two unheated elastic pressure members which progressively contact each other along a narrow band defining a nip, said members possessing moduli of elasticity compression permitting, when said members are loaded sufficiently to provide a calculated peak nip pressure in excess of the threshold pressure for the toner, deformation at said nip in an amount corresponding to a substantial multiple of the thickness variation of said workpiece; and loading said pressure members to an extent providing a calculated peak nip

pressure in excess of said threshold pressure for the toner when said workpiece is disposed between said members, and passing said workpiece through said nip between the pressure members to pressure fix said powder image upon said substrate.

2. The method defined in claim 1 wherein at least one of said pressure members has a modulus of elasticity in compression within the range of about 100,000 to about 2,000,000 p.s.i.

3. The method defined in claim 1 wherein each of said pressure members has a modulus of elasticity in compression within the range of about 100,000 to about 2,000,000 p.s.i.

4. The method defined in claim 1 wherein at least one of said pressure members has a surface formed of nylon.

5. The method defined in claim 1 wherein one of said pressure members has a surface formed of steel which is disposed to contact said powder toner image when said workpiece is passed between said pressure members.

6. The method defined in claim 1 wherein both of said pressure members have surfaces formed of nylon.

7. The method defined in claim 1 wherein one of said pressure members has a surface formed of textile material.

8. The method defined in claim 1 wherein at least one of said pressure members is a roller.

9. The method defined in claim 1 wherein both of said pressure members are rollers.

10. The method of fixing a toner image to a substrate which comprises passing the substrate with a powder toner image thereon under ambient temperature conditions between a pair of unheated pressure members progressively contacting each other along a narrow band, at least one of said members being of a somewhat compliant material having a modulus of elasticity in compression within the range of about 100,000 to about 2,000,000 p.s.i., and applying to the pressure members a loading sufficient to provide a calculated peak nip pressure in excess of the toner threshold pressure and averaging at a value within the range of about 2,000 to about 10,000 p.s.i., for as long as the toner bearing portions of the substrate are in contact with a pressure member during the passage.

11. The method defined in claim 10 wherein at least one of said pressure members has a surface formed of nylon.

12. The method defined in claim 10 wherein each of said pressure members has a surface formed of nylon.

13. The method defined in claim 10 wherein one of said pressure members has a surface formed of textile material.

14. The method defined in claim 10 wherein one of said pressure members has a chrome-plated steel surface which is disposed to contact said powder toner image when said substrate is passed between said pressure members.

15. The method defined in claim 10 wherein at least one of said pressure members is a roller.

16. The method defined in claim 10 wherein both of said pressure members are rollers.

17. Apparatus for providing a permanent image on a substrate of substantial width, wherein the image is a fixed powder image of electroscopic toner powder having a predetermined threshold pressure, comprising means for creating an electrostatic charge pattern in image configuration; means for depositing electroscopic toner powder upon said substrate to form an image pattern configuration under the electrical control of said charge pattern to create a workpiece having thickness variations; and means for fixing the toner powder image to said substrate, wherein the last mentioned means includes two unheated elastic pressure members which progressively contact each other along a narrow band defining a nip and thereby advance a workpiece therebetween, said members possessing moduli of elasticity in compression permitting, when said members are loaded sufficiently to provide a calculated peak nip pressure in excess of the threshold pressure for the toner, deformation at said nip in an amount corresponding to a substantial multiple of the thickness variation of said workpiece; and means for loading said pressure members to an extent providing a calculated peak nip pressure in excess of said threshold pressure for the toner when said workpiece is disposed between said members.

18. Apparatus for providing a permanent image on a substrate of substantial width wherein the image is a fixed powder image of electroscopic toner powder, comprising means for creating an electrostatic charge pattern in image configuration; means for depositing electroscopic toner powder upon said substrate to form an image pattern configuration under the electrical control of said charge pattern; and means for fixing the toner powder image to said substrate, wherein the last mentioned means includes a pair of unheated pressure members arranged for progressively contacting each other along a narrow band with rolling pressure contact, at least one of said members having a modulus of elasticity in compression within the range of from about 100,000 to about 2,000,000 p.s.i.; and means providing a load on said pressure members of such magnitude that there is exerted on the substrate passing therebetween a calculated pressure on the imaged substrate at the peak pressure point on its passage through the machine having an average value within the range of from about 2,000 to about 10,000 p.s.i.

19. The apparatus defined in claim 18 wherein both of said pressure members are rollers.

20. The apparatus defined in claim 19 wherein at least one of said rollers has a surface formed of nylon.

21. The apparatus defined in claim 19 wherein one of said rollers has a surface formed of a textile material.

\* \* \* \* \*

UNITED STATES PATENT OFFICE  
CERTIFICATE OF CORRECTION

Page 1 of  
two pages

Patent No. 3 854 975 Dated December 17, 1975

Inventor(s) Richard S. Brenneman, David W. Lovering, Frederick E. Barr

It is certified that error appears in the above-identified patent and that said Letters Patent are hereby corrected as shown below:

Column 1, line 8 (numbered 10), after the word "powder" there should be inserted --image--. Column 2, line 30, "or narrow" should read --of narrow--; the heading "DESCRIPTION OF THE PREFERRED EMBODIMENT" appearing in lines 57 and 58 should instead appear between lines 39 and 40. Column 3, line 12, "line of" should read --line or--; line 44, "purposed" should read --purposes--; line 48, "must" should read --most--; line 52, after "one-fourth" should be inserted --inch--; line 62, "makes is" should read --makes it--. Column 4, line 42, "elastic" should read --elasticity--. Column 6, the formula appearing in lines 4 and 5 should read:

$$b = 1.6 \sqrt{p \frac{D_1 D_2}{D_1 + D_2} \left[ \frac{1 - v_1^2}{E_1} + \frac{1 - v_2^2}{E_2} \right]}$$

Column 6, the formula appearing in lines 32 and 33 should read:

$$\text{Max. } s_c = 0.798 \sqrt{\frac{p \frac{D_1 + D_2}{D_1 D_2}}{\frac{1 - v_1^2}{E_1} + \frac{1 - v_2^2}{E_2}}}$$

UNITED STATES PATENT OFFICE  
CERTIFICATE OF CORRECTION

Page 2 of  
two pages

Patent No. 3 854 975 Dated December 17, 1975

Inventor(s) Richard S. Brenneman, David W. Lovering, Frederick E. Barr

It is certified that error appears in the above-identified patent and that said Letters Patent are hereby corrected as shown below:

Column 6, line 58, the fraction " $D_1 D_2 / D_1 + D_2$ " should read:

$$\frac{D_1 D_2}{D_1 + D_2}$$

Column 7, line 33 (numbered 36), "Pat. No. 874,811" should read --Pat. No. 874,911--; line 47 (numbered 55), "purpose" should read --pressure--. Column 9, line 13, after "characteristics," there should be inserted --this component of the variation may, as a practical matter,--; line 20, "formed" should read --forms--. Claim 1, line 15, following "elasticity" there should be inserted --in--.

Signed and sealed this 13th day of May 1975.

(SEAL)

Attest:

RUTH C. MASON  
Attesting Officer

C. MARSHALL DANN  
Commissioner of Patents  
and Trademarks